# EUROPEAN PATENT SPECIFICATION

(11) **EP 0 696 808 B1**
(45) Date of publication and mention of the grant of the patent: **17.03.1999**
(21) Application number: 95111676.3
(22) Date of filing: 25.07.1995
(51) Int. Cl.: H01B 7/00

(54) **Winding-type noise-suppressing high-tension resistive cord**
Geräuschunterdrückender Hochspannungskabel mit gewundener Widerstand
Câble haute tension à résistance enroulée et à suppression des bruits

(30) Priority: 08.08.1994 JP 186073/94
(43) Date of publication of application: 14.02.1996
(73) Proprietor: Sumitomo Wiring Systems, Ltd., Yokkaichi-City, Mie Pref. 513 (JP)
(72) Inventor: Higashikozono, Makoto, c/o Sumitomo, Yokkaichi-City, Mie Pref. 513 (JP); Kawakita, Genya, c/o Sumitomo, Yokkaichi-City, Mie Pref. 513 (JP)
(74) Representative: R.A. KUHNEN & P.A. WACKER

(56) References cited:
- EP-A- 0 329 188
- DE-A- 4 034 197

## Description

### BACKGROUND OF THE INVENTION

### Field of the Invention

The present invention relates to a winding-type noise-suppressing high-tension resistive cord to be used as an ignition cable for an internal combustion engine of an automotive vehicle and the like.

### Description of the Prior Art

High-tension resistive cords for transmitting a high voltage generated at an ignition coil to a spark plug directly or through a distributer have been required to have a low electric transmission loss, a good noise suppressing effect, and high resistance to heat and voltage. In general, currently used high-tension resistive cords are of two types: a string-type high-tension resistive cord which includes fibers impregnated with carbon; and a winding-type high-tension resistive cord which includes a metal small-gage wire having a high specific resistance and wound about a core made of a magnetic material or the like.

As shown in Fig. 3 is disclosed the winding-type high-tension resistive cord which comprises a reinforcing string 51 of aramid fibers, glass fibers or the like; a core 52 formed by extrusion-coating the reinforcing string 51 with a base polymer including ferrite powder mixed therein; a resistance wire 53 coiled around the core 52; an insulating layer 54 for extrusion-coating the core 52 and the resistance wire 53; a braid 55 for coating the insulating layer 54; and an outermost sheath 56 for coating the braid 55 (Japanese Utility Model Publication No. 1-32253 (1989)).

In this type of winding-type high-tension resistive cord, as shown in Fig. 4, the insulating layer 54 is stripped and the core 52 around which the resistance wire 53 is wound is bent along the outer surface of the cord in its longitudinal direction. Then a tubular metal terminal A is fitted on the cord, with the core 52 with the resistance wire 53 bent, for connection between the metal terminal A and the resistance wire 53. Thus, coils of the resistance wire 53 must be prevented from coming loose when the insulating layer 54 is stripped and from deviating to contact each other when the core 52 is bent which might result in changes in resistance. For this reason, it has been a common practice to coil the resistance wire 53 around the core 52, with the base polymer unvulcanized and inelastic, to embed the resistance wire 53 in the core 52, and then to vulcanize the base polymer to hold the resistance wire 53 resiliently denting the surface of the core 52.

In this type of winding-type high-tension resistive cord, the material of the core 52 generally used is fluororubber and silicone rubber which are a base polymer of high heat-resistance and high strength (Japanese Utility Model Publication No. 60-28002 (1985) and Japanese Utility Model Publication No. 5-20467 (1993)). However, the use of less expensive ethylene propylene rubber (EPR) as the base polymer of the core has been desired in place of fluororubber and silicone rubber which are costly.

The EPR used as the base polymer of the core, however, does not provide a suitable hardness when it is unvulcanized, failing to cause the resistance wire to suitably resiliently dent the surface of the core when the resistance wire is wound around the core of the unvulcanized base polymer. Further, vulcanized EPR has a low strength and low elongation, resulting in the core torn off during the removal of the insulating layer and cracks in the core when bent for connection to the terminal.

Document EP-A-0 329 188 which is considered to represent the most relevant state of the art discloses a winding-type noise-suppressing high-voltage resistive cord comprising a core, a resistance wire coiled around the core and an insulating layer for coating said core around which the resistance wire is coiled. The core is formed as ferrite rubber layer comprising a base polymer, for example ethylene-propylene, which contains ferrite powder and electrically conductive particles.

### SUMMARY OF THE INVENTION

Object of the present invention is to improve a winding-type noise-suppressing high-voltage cord according to the preamble of claim 1 in such a way that tensile strength and hardness of a core of the cord and adhesion of a resistance wire on the core are increased.

This object is solved by the advantageous measures indicated in the charactersizing part of claim 1.

Preferably, the reinforcing polymer is ethylene-vinyl acetate copolymer.

Preferably, the reinforcing polymer is polyethylene.

Preferably, the reinforcing polymer is polypropylene.

According to the winding-type noise-suppressing high-tension resistive cord of the present invention, the presence of the reinforcing polymer having the good compatibility with EPR allows the unvulcanized core to have a strength suitable to coil the resistance wire therearound. The vulcanization causes cross-linkage in the EPR, in the reinforcing polymer, and between the EPR and reinforcing polymer to increase the strength of the vulcanized core. Therefore, the winding-type noise-suppressing high-tension resistive cord having physical properties identical with those of the conventional cord including the core of fluororubber and silicone rubber is fabricated at low costs.

The object, features, aspects and advantages of the present invention will become more apparent from the following detailed description of the present invention when taken in conjunction with the accompanying drawings.

### BRIEF DESCRIPTION OF THE DRAWINGS

Fig. 1 is a perspective view of a preferred embodiment according to the present invention;
Fig. 2 is a detail sectional view of a core around which a resistance wire is wound according to the preferred embodiment;
Fig. 3 is a perspective view of the prior art; and
Fig. 4 is a sectional view illustrating connection between the prior art cord and a metal terminal.

### DESCRIPTION OF THE PREFERRED EMBODIMENT

A preferred embodiment will now be described according to the present invention with reference to the drawings. Referring to Fig. 1, a winding-type noise-suppressing high-tension resistive cord 10 comprises a reinforcing string 11 including three twisted 1000-denier aramid yarns, and a core 12 of a 1.3 mm outer diameter formed by extrusion-coating the reinforcing string 11 with a polymer including ferrite powder mixed therein.

The ferrite powder preferably includes Mn-Zn based ferrite such as Mn-Zn-Fe (manganese-zinc-ferric oxide).

The polymer is a blend of ethylene-propylene-diene terpolymer (EPDM) which is one of the EPR as a base polymer and ethylene-vinyl acetate copolymer (EVA) which is EPDM-compatible and to be covulcanized during vulcanization as a reinforcing polymer. The blend ratio of EPDM to EVA is 60 parts by weight of the former to 40 parts by weight of the latter. The core 12 contains 100 parts by weight of the blend polymer and 500 parts by weight of the ferrite powder.

A 50 µm Ni-Cr resistance wire 13 is coiled 7200 times per meter around the core 12, with the blend polymer unvulcanized. Since the unvulcanized blend polymer has a suitable hardness, the resistance wire 13 is half embedded in the core 12 as shown in Fig. 2. The resistance wire 13 is held half embedded in the core 12 by subsequent vulcanization (under conditions of 160°C.; 30 minutes).

An insulating layer 14 is formed by EPDM extrusion coating on the core 12 around which the resistance wire 13 is wound. The insulating layer 14 is coated with a reinforcing braid 15 made of glass yarn, and the reinforcing braid 15 is coated with a sheath 16 made of EPDM.

The reinforcing polymer is not limited to EVA but may be polypropylene (PP) and polyethylene (PE), for example. In particular, EVA and PE are suitable.

As shown in Table 1, when the blend ratio of EPDM to PE is within the range of about 80 to about 70 parts by weight of the former to, correspondingly, about 20 to about 30 parts by weight of the latter (that is, the blend polymer includes about 20 to about 30 % by weight of the PE) and the blend ratio of EPDM to EVA is within the range of about 80 to about 40 parts by weight of the former to, correspondingly, about 20 to about 60 parts by weight of the latter (that is, the blend polymer includes about 20 to about 60 % by weight of the EVA), satisfactory extrusion workability is obtained if about 100 to about 600 parts by weight of the ferrite powder is mixed, and the physical properties of the unvulcanized polymer are a hardness of 75 to 85 and an elongation of 50 % or more. This prevents the core 12 from being cracked when the resistance wire 13 is wound therearound and from being torn off.

Further, in the above described blend ratio ranges, the obtained physical properties of the vulcanized polymer are a strength of 5 MPa or more and an elongation of 50 % or more. This prevents the core 12 from being torn off and cracked when the insulating layer 14 is stripped and the core is bent for connection between the cord and the metal terminal.

While the invention has been shown and described in detail, the foregoing description is in all aspects illustrative and not restrictive. It is therefore understood that numerous modifications and variations can be devised without departing from the scope of the invention.

## Claims

1. A winding-type noise-suppressing high-tension resistive cord (10) comprising:
a core (12) including a polymer and a ferrite powder mixed therein;
a resistance wire (13) coiled around said core; and
an insulating layer (14) for coating said core around which said resistance wire hat first been coiled; *characterized in that*
said polymer is a blend polymer being made by blending ethylene propylene rubber as a base polymer with a reinforcing polymer having a good compatibility with the ethylene propylene rubber and having been covulcanized during vulcanization, and said resistance wire is half embedded in said core with said blend polymer being in an unvulcanized state.

2. The winding-type noise-suppressing high-tension resistive cord of claim 1, wherein
said insulating layer (14) is coated with a reinforcing braid (15) and said reinforcing braid is coated with a sheath (16).

3. The winding-type noise-suppressing high-tension resistive cord of claim 1 or 2, wherein
said reinforcing polymer is ethylene-vinyl acetate copolymer.

4. The winding-type noise-suppressing high-tension resistive cord of claim 3, wherein
said blend polymer includes about 20 to about 60 % by weight of said reinforcing polymer.

5. The winding-type noise-suppressing high-tension resistive cord of claim 1 or 2, wherein
said reinforcing polymer is polyethylene.

6. The winding-type noise-suppressing high-tension resistive cord of claim 5, wherein
said blend polymer includes about 20 to about 30 % by weight of said reinforcing polymer.

7. The winding-type noise-suppressing high-tension resistive cord of claim 1 or 2, wherein
said reinforcing polymer is polypropylene.

8. The winding-type noise-suppressing high-tension resistive cord of claim 4 or 6, wherein
said ferrite powder is mixed in an amount of about 100 to about 600 parts by weight per 100 parts by weight of said blend polymer.

## Patentansprüche

1. Gewickeltes geräuschunterdrückendes Hochspannungsfestes Kabel (10), welches aufweist:
einen Kern (12), welcher ein Polymer und ein darin vermischtes Ferritpulver aufweist;
ein Widerstandskabel (13), welches um den Kern gewickelt ist; und
eine Isolierschicht (14) zur Ummantelung des Kerns, um welchen zuerst das Widerstandskabel gewickelt worden ist,
dadurch gekennzeichnet, daß
das Polymer ein Polymergemisch ist, welches durch Mischung von Ethylen-Propylen-Gummi als Grundpolymer mit einem Verstärkungspolymer, welches eine gute Kompatiblität mit dem Ethylen-Propylen-Gummi aufweist und während einer Vulkanisierung zusammen-vulkanisiert wird, und wobei das Widerstandskabel zur Hälfte in den Kern eingebettet ist, wobei sich das Polymergemisch in einem unvulkanisierten Zustand befindet.

2. Gewickeltes geräuschunterdrückendes Hochspannungsfestes Kabel nach Anspruch 1, wobei
die Isolierschicht (14) mit einer Verstärkungsumflechtung (15) ummantelt ist und wobei die Verstärkungsumflechtung mit einer Ummantelung (16) ummantelt ist.

3. Gewickeltes geräuschunterdrückendes Hochspannungsfestes Kabel nach Anspruch 1 oder 2, wobei
das Verstärkungspolymer ein Ethylen-Vinyl-Acetat-Copolymer ist.

4. Gewickeltes geräuschunterdrückendes Hochspannungsfestes Kabel nach Anspruch 3, wobei
das Polymergemisch in etwa 20 bis in etwa 60 Gew.-% des Verstärkungspolymers aufweist.

5. Gewickeltes geräuschunterdrückendes Hochspannungsfestes Kabel nach Anspruch 1 oder 2, wobei das Verstärkungspolymer Polyethylen ist.

6. Gewickeltes geräuschunterdrückendes Hochspannungsfestes Kabel nach Anspruch 5, wobei
das Polymergemisch in etwa 20 bis in etwa 30 Gew.-% des Verstärkungspolymers aufweist.

7. Gewickeltes geräuschunterdrückendes Hochspannungsfestes Kabel nach Anspruch 1 oder 2, wobei
das Verstärkungspolymer Polypropylen ist.

8. Gewickeltes geräuschunterdrückendes Hochspannungsfestes Kabel nach Anspruch 4 oder 6, wobei
das Ferritpulver in einem Betrag von in etwa 100 bis in etwa 600 Gewichtsanteilen pro 100 Gewichtsanteilen des Polymergemisches vermischt ist.

## Revendications

1. Câble haute tension (10) antiparasite du type à résistance enroulée, comprenant :
une âme (12) comprenant un polymère et une poudre de ferrite mélangée à celui-ci,
un fil de résistance (13) enroulé autour de cette âme; et
une couche isolante (14) pour recouvrir cette âme autour de laquelle ce fil de résistance a d'abord été enroulé;
caractérisé en ce que ce polymère est un polymère de mélange qui est fait par mélange d'un caoutchouc d'éthylène-propylène en tant que polymère de base avec un polymère de renforcement qui a une bonne compatibilité avec le caoutchouc d'éthylène-propylène et qui a été covulcanisé pendant la vulcanisation, et en ce que ce fil de résistance est à moitié noyé dans cette âme avec ce polymère de mélange qui se trouve dans un état non vulcanisé.

2. Câble haute tension antiparasite du type à résistance enroulée suivant la revendication 1, dans lequel
cette couche isolante (14) est revêtue d'une tresse de renforcement (15) et cette tresse de renforcement est revêtue d'une gaine (16).

3. Câble haute tension antiparasite du type à résistance enroulée suivant les revendications 1 ou 2, dans lequel
ce polymère de renforcement est un copolymère d'éthylène et d'acétate de vinyle.

4. Câble haute tension antiparasite du type à résistance enroulée suivant la revendication 3, dans lequel
ce polymère de mélange comprend environ 20% à environ 60% en poids de ce polymère de renforcement.

5. Câble haute tension antiparasite du type à résistance enroulée suivant les revendications 1 ou 2, dans lequel
ce polymère de renforcement est un polyéthylène.

6. Câble haute tension antiparasite du type à résistance enroulée suivant la revendication 5, dans lequel
ce polymère de mélange comprend environ 20% à environ 30% en poids de ce polymère de renforcement.

7. Câble haute tension antiparasite du type à résistance enroulée suivant les revendications 1 ou 2, dans lequel
ce polymère de renforcement est un polypropylène.

8. Câble haute tension antiparasite du type à résistance enroulée suivant les revendications 4 ou 6, dans lequel
cette poudre de ferrite est mélangée à raison d'une quantité d'environ 100 à environ 600 parties en poids pour 100 parties en poids de ce polymère de mélange.
